

## United States Patent Office

2,868,294

Patented Jan. 13, 1959

1

Cement is



2,868,294

## WELL CEMENTING

Alvin F. Beale, Jr., Louis H. Eilers, and William T. Abel,  
Tulsa, Okla., assignors to The Dow Chemical Company,  
Midland, Mich., a corporation of Delaware

No Drawing. Application May 23, 1955  
Serial No. 510,575

27 Claims. (Cl. 166—29)

The invention relates to methods of and compositions for cementing. It more particularly relates to an improved method of cementing wells drilled into the earth.

In boring into the earth for oil, gas, water, or brine, it is oftentimes necessary, if not desirable, to provide a casing in the bore hole. The casing is usually in the form of a steel pipe. One of the functions of a well casing is to prevent the sides of the bore hole from caving or sloughing into the well. Another function is to provide means to collect the fluids which enter the well hole. The casing also may be used in preventing fluid from one earth stratum from entering the well while permitting inflow from another. Still other uses of the casing are made depending upon the geology of the earth region involved and the use to which the well is put. In the case of disposal wells, for example, the casing serves to direct the introduced fluid into a particular zone or zones penetrated by the well hole. The casing may extend for the entire length or only a portion of the well bore. Communication between the bore of the casing and the adjacent earth may be effected by forming perforations in the casing at appropriate levels.

The successful fulfillment of the functions of a casing in a well hole depends in general upon whether or not the space between the bore hole wall and the outside of the casing can be tightly sealed. Such sealing is necessary to prevent fluid from migrating up or down between the earth and casing. In high pressure wells, it is essential also that the casing be firmly anchored in the hole to keep it in place against the fluid pressure which tends to eject it. Heretofore the almost universal practice of attempting to seal a casing in a well hole has been to deposit in the annular space between the casing and the well hole, in one way or another, a slurry of Portland or gypsum cement and water. The slurry so-deposited is allowed to harden in situ. Although adequate seals are at times obtained, nevertheless numerous difficulties arise in the conventional cementing practice which heretofore have not been adequately overcome. These difficulties militate against achieving the desired objectives of a well cementing operation.

One of these difficulties is that the temperature of the earth formation affects the rate at which the cement slurry stiffens and hardens. In a well hole, it is not always possible to bring about suitable temperature conditions appropriate to the natural setting rate of the cement. As a consequence, severe limitations are oftentimes imposed as to the amount of time available, after the slurry is prepared, during which the slurry remains sufficiently fluid to permit placing it in position in the well as by pumping. In very deep wells, such limitations of time and setting or thickening rates oftentimes make it mandatory to perform the cementing operation in stages. This requires the use of especial equipment and is time-consuming. In any case after the cement has been manufactured and shipped to the well, its rate of setting cannot be changed much.

2

Another of the difficulties with conventional well cementing practices results from contamination of the cement injected into the well. Such contamination is due to the presence in the well hole and in the cracks, crevices, and fissures of the earth formation of material of one kind or another with which the cement slurry comes in contact. These contaminants interfere with the cementing action. Perhaps one of the most disadvantageous of these undesirable materials is the fluid with which the well may be drilled. The drilling fluid is usually present in the well hole during the cementing operation. Both the clay particles, as well as many of the drilling mud additaments (e. g. quebracho), of which drilling fluids are composed, interfere with the setting of the cement slurries. Clay mud on becoming incorporated in the cement slurry, as it is being placed in position in a conventional casing cementing operation, dilutes and weakens the cement. Clay-base drilling mud also prevents the cement from bonding to the wall of the well hole. Because of the use of mud in drilling the well, the well wall is coated more or less with a layer of mud or mud cake. In conventional cementing practice, the cement slurry is unable to assimilate the mud in either the fluid or cake form without suffering a loss in strength.

In addition, a true seal cannot be produced by the cement in the annular space outside the casing when the earth formation is more or less coated with a mud cake produced in drilling the well hole.

In conventional well cementing practice, especially in wells which are unusually deep, a high hydrostatic pressure is exerted by the cement slurry against the well hole on placing the cement slurry behind a casing. Under these conditions, the difficulty arises that a premature dehydration of the cement slurry may occur. The dehydration results from the filtering action of the earth formation. In this action, the aqueous phase of the slurry is pressed out of it into the earth formation leaving the cement excessively dry. Cement so-dehydrated becomes immobile or unpumpable. For this reason, the dehydrated cement slurry cannot be circulated into position around a casing. The high density of the cement slurry used in conventional cementing operations is a contributing factor to such premature dehydration. Attempts to maintain the cement slurry in a fluid state by agitating the slurry during the stiffening or gelling period also precludes setting with proper strength. Addition of bentonite in attempts to reduce water loss weakens conventional cement.

Some of the cements in common use in conventional well cementing are attacked by saline ground waters, especially those containing sulfate. The destruction of the cement may be brought about prematurely by contact with saline ground water.

Another difficulty in conventional well cementing practice is that the set cement, in an annular space about a casing in a well hole, does not perforate cleanly and without cracking or shattering in the vicinity of the perforation. This is a disadvantage in a well having a casing traversing, for example, a producing oil or gas zone adjacent to a water zone which is to be sealed off while obtaining production of oil or gas. In such a situation, perforating the casing opposite the oil or gas zone may result in shatter cracks extending from one level to another in the cemented annulus. Such cracks can admit unwanted water to the well.

In view of the various difficulties and problems of conventional cementing operations, it is a desideratum in the art, not only to improve the cementing practice but also to provide improved cementing materials.

Accordingly, it is the principal object of the invention to provide an improved well cementing method which overcomes many of the difficulties inherent in the conventional well cementing operations. Another object is to provide improved cementing material. Still other objects and advantages will appear as the description of the invention proceeds.

Among the discoveries on which the present invention is based is that a cement comprising phosphoric acid in admixture with an aluminous material (preferably substantially alkali free) with which it is capable of reacting, on being placed against the surface of a geological formation, such as the wall of a well hole in the earth, resists filtration, and on being permitted to set in situ becomes bonded thereto even though the surface may be more or less coated with a clay. Further it has been discovered that by including in the cement comprising phosphoric acid and the aluminous material certain additaments of a more or less water-soluble character new properties are developed which are especially advantageous in forming sealing deposits in the earth, as in cementing a pipe in a well hole. Among the additaments contemplated by the invention are water-soluble fluorides, particularly the alkali metal and ammonium fluorides and bifluorides, for example,  $\text{NH}_4\text{F}$ ,  $\text{NH}_4\text{F}\cdot\text{HF}$ ,  $\text{KF}$ ,  $\text{KF}\cdot 2\text{H}_2\text{O}$ ,  $\text{KF}\cdot\text{HF}$ , as well as HF or hydrofluoric acid. These aid in determining and controlling the rate at which setting may be brought about. The soluble fluorides improve the tolerance of the cement for contaminating agents, such as drilling muds and drilling mud additaments normally having an adverse action of the setting and cementing characteristics of conventional oil well cements. The soluble fluorides also improve strength and bring about resistance to the softening action of heat, experienced to a greater or less extent with the cements made with phosphoric acid and the non-siliceous substantially pure aluminous materials, e. g. gibbsite, but not containing the soluble fluoride additament. Complex more or less water-soluble fluorides also may be used to accelerate the rate of set, especially at the higher temperatures encountered in the deeper wells currently being drilled, for example,  $\text{K}_2\text{TiF}_6$ ,  $\text{K}_2\text{SiF}_6$ ,  $\text{KPF}_6$ ,  $(\text{NH}_4)_2\text{SiF}_6$ ,  $\text{K}_3\text{CrF}_6$ ,  $\text{KBF}_4$ ,  $\text{HPO}_2\text{F}_2$ ,  $\text{H}_2\text{PO}_3\text{F}$ ,  $\text{HPPF}_6$ ,  $(\text{NH}_4)_2\text{TiF}_6$ .

The presence of the ions of potassium and ammonium

are especially advantageous in improving the properties and cementing action in mudded well bores of the cements comprising phosphoric acid and the aluminous material, especially when in the presence of a fluoride.

5 Suitable sources of potassium ion are water-soluble inorganic potassium salts in addition to the potassium compounds listed above, for example, potassium sulfate, potassium phosphate, potassium hydroxide, potassium chromate and potassium bichromate. The corresponding ammonium salts may be used as a source of ammonium ion.

10 The invention then consists of the improved method of cementing particularly against an earth formation with settable mixtures comprising an aluminous material and phosphoric acid, including improved compositions thereof, herein fully described and particularly pointed out in the claims.

15 In carrying out the invention, a cement is prepared with one or more suitable aluminous materials, in particulate form, capable of undergoing a cement-forming reaction with phosphoric acid in the presence of water. A wide variety of aluminous materials are capable of undergoing the desired reaction with phosphoric acid, including the various aluminum oxides, aluminum hydroxides, and aluminum silicates. These materials are generally water-insoluble and contain more than 10 percent by weight of alumina calculated as  $\text{Al}_2\text{O}_3$ . For reasons of cost and availability, many of the naturally occurring aluminous minerals may be used, as the aluminous material, without purification and with a minimum of processing. Generally milling and drying or calcining suffices to prepare naturally occurring aluminous materials for use. Bauxite, kaolin, and kaolinitic clays are especially suitable. Common clays containing at least 10 percent of  $\text{Al}_2\text{O}_3$  on the dry basis may be used. The use of an aluminum silicate or aluminum silicate-containing material as the aluminous material has the advantage of rendering the cements resistant to heat-softening at the elevated temperatures encountered in deep wells.

20 40 The following Table I sets forth a number of examples of aluminous materials which may be used. They may be ground or otherwise comminuted before use, if necessary. The particle size does not appear to be sharply critical, but is preferably at least as fine as that mostly

25 30 35 40 45 passing through a number 40 standard sieve.

Table I

| No. | Aluminous Material         | Analysis, Percent by Weight |                |                      |                         |                |              | Percent Ignition Loss | Sieve No. <sup>1</sup> | Remarks: Source         |
|-----|----------------------------|-----------------------------|----------------|----------------------|-------------------------|----------------|--------------|-----------------------|------------------------|-------------------------|
|     |                            | $\text{Al}_2\text{O}_3$     | $\text{SiO}_2$ | $\text{H}_2\text{O}$ | $\text{Fe}_2\text{O}_3$ | $\text{TiO}_2$ | Other Oxides |                       |                        |                         |
| 1.  | Corundum                   | 99                          |                |                      |                         |                | 1            | <1                    | -100                   |                         |
| 2.  | Activated alumina          | 92                          | 1              | 7                    |                         |                |              | 7                     | -100                   | 47 heated at 1,200 °F.  |
| 3.  | Aluminum hydroxide         | 65                          | 0              | 35                   |                         |                |              | 35                    | -325                   |                         |
| 4.  | Aluminum oxide trihydrate  | 65                          | 0              | 35                   |                         |                |              | 35                    | -200                   |                         |
| 5.  | do                         | 57                          | 2              | 39                   | <1                      |                | <1           | 40                    | 0.5 micron             |                         |
| 6.  | do                         | 65                          | 0              | 35                   |                         |                | <1           | 35                    | 0.5 micron             |                         |
| 7.  | do                         | 65                          | 0              | 35                   |                         |                |              | 35                    | -100                   |                         |
| 8.  | Bauxite                    | 59                          | 14             | 23                   | 2                       | 2              |              | 27                    | -40                    |                         |
| 9.  | do                         | 58                          | 12             | 25                   | 3                       | 2              |              | 25                    | -100                   | Pulaski Co., Ark.       |
| 10. | do                         | 54                          | 13             | 25                   | 2                       | 2              | 2            | 24.5                  | -40                    | Purified.               |
| 11. | do                         | 55                          | 7              | 28                   | 3                       | 2              | 4            | 30                    | -40                    | Eufaula, Ala.           |
| 12. | do                         | 54                          | 11             | 28                   | 3                       | 2              | 2            | 30                    | -40                    | Saline Co., Ark.        |
| 13. | do                         | 52                          | 2              | 25                   | 15                      |                | 6            | -40                   | Pulaski Co., Ark.      |                         |
| 14. | do                         | 52                          | 1              | 23                   | 20                      |                | 4            | -40                   | Do.                    |                         |
| 15. | do                         | 52                          | 16             | 25                   | 4                       | 2              | 1            | -40                   | Jamaica.               |                         |
| 16. | do                         | 50                          | 15             | 25                   | 6                       | 3              | 1            | -40                   | Saline Co., Ark.       |                         |
| 17. | do                         | 50                          | 14             | 26                   | 7                       | 2              | 1            | -40                   | Do.                    |                         |
| 18. | Bauxitic clay              | 47                          | 24             | 23                   | 2                       | 2              | 2            | -40                   | Pulaski Co., Ark.      |                         |
| 19. | do                         | 45                          | 30             | 21                   | 1                       | 2              | 1            | -40                   | Do.                    |                         |
| 20. | Kaolinitic clay            | 43                          | 33             | 19                   | 2                       | 2              | 1            | 20                    | -40                    | Saline Co., Ark.        |
| 21. | do                         | 42                          | 36             | 19                   | 1                       | 2              |              | 20                    | -40                    | Pulaski Co., Ark.       |
| 22. | do                         | 37                          | 45             | 14                   | 2                       | 1              | 1            | 16                    | -40                    | Do.                     |
| 23. | Kaolinitic clay, activated | 41                          | 50             | 5                    |                         |                | 4            | 5                     | -40                    | Do.                     |
| 24. | Kaolinitic clay, calcined  | 43                          | 53             | 0                    |                         |                | 4            | 0                     | -40                    | #22 heated to 2,400 °F. |
| 25. | Illitic clay               | 42                          | 44             | 10                   | 1                       | 1              | 2            | 10                    | -40                    | Texas.                  |
| 26. | Kaolinite                  | 39.5                        | 46.5           | 14                   |                         |                |              | 14                    | -40                    |                         |
| 27. | Muscovite                  | 39                          | 45             | 3                    |                         |                | 12           | 3                     | -325                   |                         |
| 28. | Anorthite                  | 37                          | 43             |                      |                         |                | 20           | 0                     | -40                    | Grass Valley, Calif.    |

Table I—Continued

| No. | Aluminous Material       | Analysis, Percent by Weight    |                  |                  |                                |                  |              |      | Percent Ignition Loss | Sieve No. <sup>1</sup> | Remarks: Source  |
|-----|--------------------------|--------------------------------|------------------|------------------|--------------------------------|------------------|--------------|------|-----------------------|------------------------|------------------|
|     |                          | Al <sub>2</sub> O <sub>3</sub> | SiO <sub>2</sub> | H <sub>2</sub> O | Fe <sub>2</sub> O <sub>3</sub> | TiO <sub>2</sub> | Other Oxides | Bal. |                       |                        |                  |
| 29  | Laboradorite             | 32                             | 50               |                  |                                |                  | 18           |      |                       | —40                    | Essex Co., N. Y. |
| 30  | Clay                     | 31                             | 54               | 11               | 2                              | 1                | 5            | 11   | —40                   | Albany Co., Wyo.       |                  |
| 31  | Anorthosite (plio-clase) | 27                             | 53               | 1                |                                | 15               |              |      | 2                     | —40                    |                  |
| 32  | Clay                     | 21                             | 59               | 10               | 4                              |                  | 4            | 11   | —40                   | Texas.                 |                  |
| 33  | Bentonite                | 20                             | 60               | >5               | <10                            | >10              | <15          | 2    | —200                  | Blackhills, So. Dak.   |                  |
| 34  | Anorthoclase             | 19                             | 68               |                  |                                |                  | 13           |      | —40                   | Larvik, Norway.        |                  |
| 35  | NaK Feldspar             | 19                             | 67               |                  |                                |                  | 14           |      | —40                   |                        |                  |
| 36  | Nepheline syenite        | 20                             | 58               | 1                | >5                             | <10              |              | 2    | —40                   | Pulaski Co., Ark.      |                  |
| 37  | Microcline               | 18                             | 65               | 0                |                                |                  | 17           |      | —40                   | Amelia Co., Va.        |                  |
| 38  | Orthoclase               | 18                             | 65               | 0                |                                |                  | 17           |      | —40                   | Kokomo, Col.           |                  |
| 39  | Clay                     | 16                             | 63               | 10               | 2                              |                  | 2            | 15   | —40                   | Texas.                 |                  |
| 40  | Biotite                  | 10                             | 47               | 1                | 15                             |                  | 20           | 2    | —40                   |                        |                  |
| 41  | Sepiolite (vermiculite)  | 7                              | 45               | 20               |                                |                  | 27           | 1    | —40                   | Lincoln Co., Mont.     |                  |
| 42  | Fuller's earth           | 12                             | 60               | 12               | 3                              |                  | 12           | 1    | 11.9                  | —100                   | Georgia.         |
| 43  | Bauxite                  | 56                             | 11               | 26               | 4                              | 3                |              | 26   | —40                   | Pulaski Co., Ark.      |                  |

<sup>1</sup> Standard screen scale; minus sign means particles pass through sieve of number indicated.<sup>2</sup> Approximate particle size.

As will be apparent from the examples given in Table I, the aluminous material may contain, as by chemical analysis, not less than about 7 percent of Al<sub>2</sub>O<sub>3</sub>. The balance of the material may involve silica, in amount not exceeding about 70 percent, Fe<sub>2</sub>O<sub>3</sub> not exceeding about 20 percent, TiO<sub>2</sub> not exceeding about 10 percent, and other metal oxides normally comprising aluminous minerals, such as CaO, MgO, K<sub>2</sub>O, Na<sub>2</sub>O, in various amounts not exceeding about 30 percent, with or without minor amounts not exceeding about 10 percent of unspecified constituents. Water may also be present in various amounts depending upon the nature and treatment, if any of the aluminous material and may amount to as much as about 40 percent of the weight of the undried aluminous material. Excessive amounts of water are not desirable and in some cases the aluminous material may require more or less drying to avoid overloading the cement mixtures with water as will be apparent in what follows.

The aluminous material, phosphoric acid, and an appropriate amount of water as needed, are mixed together in any convenient manner to form a flowable slurry. The relative amounts of aluminous material and phosphoric acid may be varied over a wide range. The proportions are chosen with reference to the rate at which the slurry is to stiffen and become a monolithic body under the environmental conditions of temperature and pressure that are involved. The temperature, water concentration, and

nature of the aluminous material affect the rate of set. The most rapid rates of setting are obtained with the aluminous hydroxides and hydrates, the aluminum silicates or clays produce slower setting cements, and the calcined aluminous materials, e. g. corundum, and dead burned clays (2400° F.), the slowest. Unless the environment in which the cement is to set is relatively warm as in the deeper wells bauxite is the preferred aluminous material to employ. The particular aluminous material used does not greatly affect the ultimate strength of the cement when the other ingredients of the cement-forming mixture are appropriate.

In general the relative amount of aluminous material and phosphoric acid to produce a cement having the setting time and strength desired can be determined by trial. A trial can be made by mixing batches of the aluminous material with various amounts of phosphoric acid diluted to various concentrations with water and setting aside the resulting mixtures at a temperature at which the cementing operation is to be performed.

As illustrative of this, commercial phosphoric acid (85 percent H<sub>3</sub>PO<sub>4</sub>, balance H<sub>2</sub>O) may be diluted with water, if necessary, and to the resulting solution, while stirring, is added the aluminous material in pulverulent form to make a slurry or cream of flowable consistency. A number of examples of cement formulations so made which are pumpable are set forth in Table II using some of the aluminous materials from Table I.

Table II

| Mix. No. | Aluminous Material |           | Lbs. 85% H <sub>3</sub> PO <sub>4</sub> | Water      |            | Ratios |                          | Setting Time at 175° F., Hours |  |  |
|----------|--------------------|-----------|-----------------------------------------|------------|------------|--------|--------------------------|--------------------------------|--|--|
|          | No. in Table I     | Lbs. Used |                                         | Lbs. Added | Total Lbs. | Al/P   | Total H <sub>2</sub> O/P |                                |  |  |
|          |                    |           |                                         |            |            |        |                          |                                |  |  |
| 1        | 6                  | 36.9      | 7.0                                     | 56.1       | 70         | 7.8    | 63.6                     | 20                             |  |  |
| 2        | 6                  | 27.7      | 14.1                                    | 58.2       | 70         | 2.9    | 31.8                     | >1 <18                         |  |  |
| 3        | 6                  | 23.1      | 17.7                                    | 59.2       | 70         | 1.9    | 25.4                     | >1 <18                         |  |  |
| 4        | 6                  | 18.5      | 21.2                                    | 60.3       | 70         | 1.3    | 21.1                     | >2 <18                         |  |  |
| 5        | 6                  | 49.3      | 9.4                                     | 41.3       | 60         | 7.7    | 40.9                     | 2                              |  |  |
| 6        | 6                  | 37.0      | 18.8                                    | 44.2       | 60         | 2.9    | 20.4                     | 5                              |  |  |
| 7        | 6                  | 27.8      | 26.0                                    | 46.2       | 60         | 1.6    | 14.8                     | 7                              |  |  |
| 8        | 6                  | 26.4      | 26.9                                    | 46.7       | 60         | 1.5    | 14.8                     | >6 <24                         |  |  |
| 9        | 6                  | 24.6      | 28.2                                    | 47.2       | 60         | 1.3    | 13.6                     | 5                              |  |  |
| 10       | 6                  | 61.6      | 11.8                                    | 26.6       | 50         | 7.7    | 27.0                     | >0.5 <16                       |  |  |
| 11       | 6                  | 53.9      | 17.7                                    | 28.4       | 50         | 4.5    | 18.1                     | >0.5 <16                       |  |  |
| 12       | 6                  | 38.5      | 29.4                                    | 32.1       | 50         | 1.9    | 10.9                     | 3                              |  |  |
| 13       | 6                  | 27.0      | 38.2                                    | 34.8       | 50         | 1.0    | 8.4                      | 18                             |  |  |
| 14       | 6                  | 23.1      | 41.2                                    | 35.7       | 50         | 0.8    | 7.8                      | 24                             |  |  |
| 15       | 2                  | 52.8      | 47.2                                    | 37.0       | 47.8       | 2.3    | 6.5                      | >0.5 <16                       |  |  |
| 16       | 2                  | 63.0      | 37.0                                    | 38.3       | 48.3       | 3.6    | 8.4                      | <0.5 <16                       |  |  |
| 17       | 10                 | 104.0     | 61.2                                    | 34.8       | 70         | 2.1    | 7.8                      | >3 <18                         |  |  |
| 18       | 10                 | 120.0     | 66.8                                    | 57.0       | 97.1       | 2.3    | 9.3                      | >4 <5                          |  |  |
| 19       | 10                 | 80.0      | 47.1                                    | 72.9       | 100.0      | 2.1    | 13.6                     | >3 <18                         |  |  |
| 20       | 10                 | 85.3      | 18.8                                    | 95.8       | 120.0      | 5.7    | 40.8                     | >4 <18                         |  |  |
| 21       | 21                 | 74.1      | 47.1                                    | 78.8       | 100.0      | 1.5    | 13.6                     | >26 <42                        |  |  |
| 22       | 21                 | 79.0      | 18.8                                    | 102.2      | 120.0      | 4.0    | 40.9                     | 92                             |  |  |
| 23       | 22                 | 96.0      | 66.8                                    | 57.0       | 80.5       | 1.2    | 7.7                      | >21 <24                        |  |  |
| 24       | 31                 | 78.9      | 61.2                                    | 60.0       | 70.0       | 0.8    | 7.3                      | 26                             |  |  |
| 25       | 31                 | 60.6      | 47.1                                    | 92.3       | 100.0      | 0.8    | 13.6                     | >26 <42                        |  |  |
| 26       | 31                 | 60.0      | 9.9                                     | 14.1       | 16.2       | 3.7    | 10.5                     | >2 <24                         |  |  |

Referring to Table II, the first column lists the mixture number; the second column the number corresponding to that in column 1, Table I, identifying the aluminous material used; the third column the number of pounds of the aluminous material used; the fourth column the number of pounds of 85 percent phosphoric acid used (85 parts by weight  $H_3PO_4$ , 15 parts by weight water); the fifth column the number of pounds of water added (exclusive of that present in the aluminous material, if any, and in the phosphoric acid solution); the sixth column the total number of pounds of water in the mixtures including that in the aluminous material, in the phosphoric, and the additional water of column 5; the seventh column the ratio of the number of moles of aluminum (Al) to the number of moles of phosphorus (P) in the mixtures; the eighth column the ratio of the number of moles of water ( $H_2O$ ) of column six to the number of moles of phosphorus (P); and the ninth column lists the setting time in hours.

In Table II, the setting time of the mixtures is the time elapsed after making the mixtures until they acquire an initial set. This initial set is that determined by the apparatus of the "vici setting-time test" in accordance with the "API recommended practice for testing oil-well cements" (API RP 10B, third edition, April 1953, issued by API Division of Production, 300 Corrigan Tower Building, Dallas 1, Texas). In making the tests for setting time, mixtures to be tested are prepared as described herein and placed in the vici mold. The mold containing the mixture is maintained at the testing temperature and periodically the mold with the mixture is given the vici-setting test above mentioned until setting is found to have occurred. Setting occurs over a wide range of ratios of moles of Al per mole of P in the mixtures which are dilute enough to be flowable yet not so dilute as to fail to set.

In simple pumpable mixtures, i. e. those involving an aluminous material, phosphoric acid, and water without modifying additaments, the ratio of the number of moles of aluminum (Al) to the number of moles of phosphorus (P) in the mixtures may range from about 0.5 to 20 with various amounts of water ranging from about 1.8 to 64 moles of water ( $H_2O$ ) per mole of phosphorus (P) in the mixtures. A preferred range of the Al to P ratio in the mixtures is from 0.8 to 3. Within this range of Al/P ratios the preferred  $H_2O/P$  ratio ranges from about 5 to 22, where the temperatures encountered by the mixtures are not over about 200° F., and about 1.8 to 10 where the temperatures encountered exceed about 200° F. Similar ratios may prevail in mixtures containing additaments herein mentioned.

Although some separation of liquid from the solids in the cement mixtures may occur as the cement mixtures set, this is an advantage in environments comprising aluminous materials, such as clays, as in most well bores. The liquid separating from the cementing mixtures when containing free phosphoric acid and particularly soluble fluoride, we have found, is capable of combining with the clays to harden them into a cement-like mass so that the separation of liquid from the cementing mixture assists in obtaining a cementitious bond with the earth formation.

Elevating the temperature of the mixtures of Table II facilitates their setting but softening results on overheating the mixtures in which the aluminous material is an oxide, hydrated oxide, or hydroxide, especially when the ratio of  $H_2O/P$  is relatively low. Softening, if any, of the cement formulations is determined by noting the rate at which one end of a  $\frac{1}{4}$  inch round rod sinks into one end of a cylindrical specimen of the set cement. The test may be carried out at various temperatures with a specified loading of the rod. In making a test of this kind, the specimen is held in a cylindrical recess in a metal block, the recess having a size which is just suffi-

cient to admit the specimen. The temperature of the block and specimen is raised at the rate of 2 to 5 degrees per minute and the rod, loaded to a weight of 150 grams, is suitably supported in a vertical position so as to rest its weight upon the specimen. An additional load of about 2 pounds is applied periodically during the test, in order to break through any crust that may form on the surface of the specimen. Softening, according to this test, is considered to have occurred when the rod, loaded to a total weight of 150 grams, sinks into the specimen below the crust, if any, at the rate of  $\frac{1}{16}$  inch per minute.

After the mixtures acquire an initial set, they are capable of supporting a compressive load and the compressive strength gradually increases with age until full strength is reached. The mixtures will set under petroleum oil, water, or brine encountered in the earth. The rate of hardening under petroleum oil is greater than that under either water or brine. Brines saturated with  $H_2S$ , often encountered in formations penetrated by oil wells, do not adversely affect the rate of hardening of the cement mixtures. The compressive strength of some of the mixtures of Table II, at moderately elevated temperature, are set forth in Table III together with the hours of ageing.

Table III

| Test No. | Table II<br>Mixture<br>No. | Setting<br>Temp.,<br>° F. | Hours of<br>Ageing | Compressive<br>Strength in<br>Lbs. Per<br>Square Inch |
|----------|----------------------------|---------------------------|--------------------|-------------------------------------------------------|
| 1.....   | 17                         | 175                       | 42                 | 4,140                                                 |
| 2.....   | 17                         | 175                       | 90                 | 4,460                                                 |
| 3.....   | 18                         | 130                       | 160                | 2,780                                                 |
| 4.....   | 18                         | 175                       | 77                 | 2,200                                                 |
| 5.....   | 19                         | 175                       | 42                 | 465                                                   |
| 6.....   | 20                         | 175                       | 42                 | 140                                                   |
| 7.....   | 23                         | 175                       | 72                 | 700                                                   |
| 8.....   | 26                         | 175                       | 24                 | 300                                                   |

Thus by formulating a mixture comprising phosphoric acid and a suitable aluminous material, as exemplified in Table II, and injecting the mixture into the annular space between a casing and the well hole in which the casing is placed, before the mixture acquires an initial set, and then allowing the injected mixture to age in situ the mixture acquires a desirable strength, as indicated in Table III, and seals the casing in place securely to the earth formation.

In some instances, as when it is desired to reduce the cost of the cementing operation, fillers may be incorporated in the mixtures. The fillers have little or no effect on the rate of setting but produce desirable effects, other than mere dilution, such as reduction of density when a light filler is used, e. g. coal, and increase in compressive strength when strong fillers are used, e. g. sand. Besides sand, and all kinds of powdered coal, powdered glass and like particulated inorganic solid materials, which are not adversely reactive with either the phosphoric acid or the aluminous material, may be used as well as ground nut shells, gilsonite, wood dust, coffee grounds, leather fiber, blast furnace dust, coke, comminuted Bakelite, and the like. In very deep wells, it is oftentimes advantageous to employ a relatively low density filler, such as pulverized bituminous coal, so as to reduce the hydrostatic head created by a long column of the fluid cement formulation which may be present in the well in a cementing operation, thereby reducing fluid and slurry loss. In the following Table IV, examples of cement formulations of the type illustrated in Table II are set forth in which fillers of sand and powdered coal have been added. The resulting mixtures are pumpable and thus capable of being pumped into position in a well hole about a casing therein set.

Table IV

| Mix No. | Aluminous Material |             | Lbs. 85% H <sub>3</sub> PO <sub>4</sub> | Water        |              | Filler       |              | Ratios |                          | Setting Time at 175° F., Hours |
|---------|--------------------|-------------|-----------------------------------------|--------------|--------------|--------------|--------------|--------|--------------------------|--------------------------------|
|         | No. in Table I     | Pounds Used |                                         | Pounds Added | Total Pounds | Coal, Pounds | Sand, Pounds | Al/P   | Total H <sub>2</sub> O/P |                                |
| 27      | 6                  | 26.4        | 26.9                                    | 46.8         | 60           | 208          | 1.4          | 14.3   | >4 <5                    |                                |
| 28      | 6                  | 26.4        | 26.9                                    | 46.8         | 60           | 88           | 1.4          | 14.3   | >7 <23                   |                                |
| 29      | 6                  | 36.9        | 7.0                                     | 56.0         | 70           | 163.2        | 7.8          | 63.6   | 43.6                     |                                |
| 30      | 6                  | 36.9        | 7.0                                     | 56.0         | 70           | 11.2         | 7.8          | 63.6   | >4 <20                   |                                |
| 31      | 6                  | 18.5        | 21.2                                    | 60.3         | 70           | 244.8        | 1.3          | 21.1   | >2 <18                   |                                |
| 32      | 6                  | 18.5        | 21.2                                    | 60.3         | 70           | 112.8        | 1.3          | 21.1   | >7 <23                   |                                |

As previously indicated, overheating the heat-softenable mixture leads to softening or even inhibition of setting. In relatively shallow wells or in wells, the earth formations of which are only moderately hotter than surface temperatures, the simple cement formulations illustrated in Table II suffice to cement the casing. On the other hand, when softening of the cement due to the ele-

amount which may be determined by trial according to 15 the rate of setting desired.

The following Table VI sets forth examples of mixtures containing other fluorides showing the composition, the rate of setting, and the compressive strength after 20 ageing the mixtures. The temperatures are representative of those encountered in the earth at various depths.

Table VI

| Mix. No. | Composition of Mixtures |           |                                         |                                       |      |            |            |        | Setting Time             | Compressive Strength |      |      |           |      |          |
|----------|-------------------------|-----------|-----------------------------------------|---------------------------------------|------|------------|------------|--------|--------------------------|----------------------|------|------|-----------|------|----------|
|          | Aluminous Material      |           | Lbs. 85% H <sub>3</sub> PO <sub>4</sub> | Soluble Fluoride                      |      | Water      |            | Ratios |                          |                      |      |      |           |      |          |
|          | No. in Table I          | Lbs. Used |                                         | Kind                                  | Lbs. | Lbs. Added | Lbs. Total | Al/P   | Total H <sub>2</sub> O/P | F/P                  | ° F. | Hrs. | Age, Hrs. | ° F. | P. s. i. |
| 35       | 1                       | 250       | 118                                     | KF.2H <sub>2</sub> O...               | 50   | 82.1       | 119.1      | 4.8    | 6.5                      | 0.52                 | 175  | 28   | 72        | 250  | 2,800    |
| 36       | 4                       | 20        | 28.7                                    | AlF <sub>3</sub> .H <sub>2</sub> O... | 10   | 0          | 13.0       | 1.0    | 2.9                      | 1.18                 | 175  | 1    | 72        | 175  | 5,000    |
| 37       | 4                       | 20        | 25.3                                    | Na <sub>3</sub> AlF <sub>6</sub> ...  | 10   | 0          | 10.8       | 1.2    | 2.7                      | 1.3                  | 175  | 0.5  | 18        | 175  | 4,400    |
| 38       | 9                       | 35        | 11.8                                    | NH <sub>4</sub> HF <sub>2</sub> ...   | 2.25 | 8.2        | 18.7       | 3.9    | 10.2                     | 0.77                 | 75   | 2    | 76        | 72   | 4,000    |
| 39       | 4                       | 64        | 15.1                                    | 50% HF...                             | 11   | 9.9        | 40.1       | 6.3    | 16.9                     | 2.1                  | 75   | 3    | 72        | 76   | 2,900    |

vated temperature of the environment cannot be tolerated, we have found, softening can be controlled by including in the cement mixtures a soluble fluoride. The addition of soluble fluoride has the advantage also of increasing the strength and bringing about setting at temperatures at which, in the absence of soluble fluoride, the mixtures exhibit undesirably long setting times. The presence of soluble fluoride can be used to modify the rate of setting to suit the case in hand and thus increases the range of usefulness of cement formulations comprising the aluminous material and phosphoric acid.

In the mixtures, as for example those of Table VI, the 40 fluorine content, derived from the fluoride, may vary over a wide range in relation to the phosphorus content which is derived from the phosphoric acid. This relation is expressed by the F/P ratio, as already indicated. This ratio may range, for example, from 0, when no fluoride is added, up to about 10 depending upon the rate of setting desired at the temperature at which the mixtures are to set and age-harden. A preferred range is from 0.025 to 2.0 for the ratio F/P.

Small amounts of soluble fluoride suffice to overcome

Table V

| Mix No.  |         | Fluoride Added |                  | Ratios |                    |      | Setting Time |            |
|----------|---------|----------------|------------------|--------|--------------------|------|--------------|------------|
| Table II | Table V | Lbs.           | Kind             | Al/P   | H <sub>2</sub> O/P | F/P  | Hours        | Temp., °F. |
| 15       | 33      | 0              | KHF <sub>2</sub> | 2.3    | 6.5                | 0    | >0.5 <16     | 175        |
| 18       | 34      | 12             | KHF <sub>2</sub> | 2.3    | 6.5                | 0.77 | 3            | 130        |
|          |         | 12             | KHF <sub>2</sub> | 2.3    | 9.3                | 0    | >4 <5        | 175        |
|          |         | 12             | KHF <sub>2</sub> | 2.3    | 9.3                | 0.52 | 0.5          | 130        |

In Table V mix numbers 33 and 34 are examples showing the effect of a soluble fluoride in shortening the setting time of mixes 15 and 18, respectively, of Table II. By the addition of a soluble fluoride setting of the phosphoric acid-aluminous material-water mixtures is brought about more rapidly and at a lower temperature. By varying the ratio of the number of moles of fluorine (F) per mole of phosphorus (P) in the mixtures different rates of setting may be obtained. In the examples given in Table V, the ratio of the numbers of moles of fluorine to the number of moles of phosphorus in the mixes is given as 0.52 in the column headed F/P. Other water-soluble inorganic fluorides may be used similarly in an

65 the heat softening characteristic of the mixtures made with those aluminous materials which yield heat-softenable mixtures. For example, from about 0.4 to 3 percent fluorine, derived from a water-soluble fluoride, suffices to control heat softening.

Similar results are obtainable by using a relatively insoluble fluoride, such as aluminum fluoride or calcium fluoride (CaF<sub>2</sub>) together with a more or less stoichiometrical equivalent amount of an acid, such as sulfuric acid, or other soluble sulfate, such as K<sub>2</sub>SO<sub>4</sub> or Al<sub>2</sub>(SO<sub>4</sub>)<sub>3</sub>, capable of decomposing the fluoride to liberate in the mixture the soluble fluoride constituent. 70 Examples of mixtures employing a fluoride, e. g. CaF<sub>2</sub>, de-

composable by a soluble sulfate are set forth in Table VII. The formulations may contain 2 percent or less to as much as 20 percent by weight of such fluoride.

Table VII

| Mix. No.        | Composition of Mixtures |           |                                         |                  |      |                                                                    |      |            |            |        |                          |      | Setting Time |        |
|-----------------|-------------------------|-----------|-----------------------------------------|------------------|------|--------------------------------------------------------------------|------|------------|------------|--------|--------------------------|------|--------------|--------|
|                 | Aluminous Material      |           | Lbs. 85% H <sub>3</sub> PO <sub>4</sub> | Fluoride         |      | Sulfate                                                            |      | Water      |            | Ratios |                          |      |              |        |
|                 | No. in Table I          | Lbs. Used |                                         | Kind             | Lbs. | Kind                                                               | Lbs. | Lbs. Added | Lbs. Total | Al/P   | Total H <sub>2</sub> O/P | F/P  | ° F.         | Hours  |
| 40 <sup>1</sup> | 22                      | 2,400     | 1,671                                   | CaF <sub>2</sub> | 750  | H <sub>2</sub> SO <sub>4</sub>                                     | 342  | 1,450      | 2,010      | 1.2    | 7.7                      | 1.32 | 175          | 72     |
| 41              | 12                      | 41.3      | 24.1                                    | CaF <sub>2</sub> | 8.4  | K <sub>2</sub> SO <sub>4</sub>                                     | 6.3  | 34.6       | 49.8       | 2.1    | 13.2                     | 1.03 | 80           | >2 <17 |
| 42              | 21                      | 42.0      | 31.2                                    | CaF <sub>2</sub> | 3.0  | Al <sub>2</sub> (SO <sub>4</sub> ) <sub>3</sub> ·6H <sub>2</sub> O | 3.0  | 26.8       | 39.4       | 1.3    | 8.0                      | 0.28 | 175          | >2 <15 |

<sup>1</sup> Mix contains 6 pounds of As<sub>2</sub>O<sub>3</sub> as a corrosion inhibitor and 45 pounds of the sodium salt of a condensed naphthalene sulfonic acid as a dispersant.

In preparing the cementing mixtures containing a soluble fluoride or having soluble fluoride-yielding material therein, the aluminous material may be mixed with the phosphoric acid solution suitably diluted, if at all, with water first and then the fluoride constituent may be added. If the fluoride constituent is water-soluble, it may be put into solution in water or in the requisite amount of diluted phosphoric acid and the solution then mixed with the aluminous material. In making such mixtures, it is apparent that some of the water may be added as a constituent of the soluble fluoride solution, if such be used, some as a constituent of the aluminous material, if not anhydrous, and the balance of the water, if any, as liquid water. However the water is present in or added to the mixtures so-made, due account must be taken of the total amount of water so that desirable H<sub>2</sub>O/P ratios are not exceeded.

It is a feature of the invention that by setting the cements against the earth formation, as in a muddled well bore, bonding to the earth by the set cement takes place. This enables a true seal to be obtained between the casing of a well and the earth formation in which it is cemented. The presence of fluoride in the cement formulation, especially when the fluoride is added as a potassium or ammonium fluorine salt, enhances the bonding. Advantageous results as regards bonding are obtained by the inclusion of sufficient fluoride in the mixtures to produce therein, in general, a fluorine-phosphorus ratio, F/P, of 0.02 to 10. Preferred ratios of F/P are about 0.1 to 2.

The following Table VIII sets forth examples of cement formulations and the strength of the bond obtained in accordance with the test described below.

In obtaining a measure of the strength of the bond, securing the cements to the surface of an earth formation, tests were made with the mixes of Table VIII. In the

tests cores of natural sandstone were used to simulate an earth formation. The cores had a permeability of approximately 2 millidarcys. The cores were cylindrical in form 3.5 inches in diameter and 10 inches long. For the tests the cores were prepared as follows. A hole 1.25 inches in diameter was bored into one end to a depth of 8 inches along the longitudinal axis. The wall of the hole was coated with a mud cake formed by forcing into the hole an aqueous drilling mud. By weight, the mud was composed of bentonite 4.4 percent, crude sodium tannate 1.0 percent, sodium hydroxide 2.0 percent, the balance being water. The mud had the following properties:

Marsh funnel viscosity----- 41 seconds.  
Fluid loss----- 9 ml. per 30 min.  
Density----- 8.7 lbs./gal.

While forcing the foregoing mud into the hole, the core was supported in a pipe nipple 4 inches in diameter with the space between the core and the inside of the nipple filled with sand. A pressure of 100 p. s. i. was maintained on the mud in the core for one hour. Bentonite was thereby filtered from the mud by the core forming a cake upon the wall of the hole. The liquid portion of the mud thus filtered out seeped into or through the core into the sand around it. After forming the mud cake, the fluid mud remaining in the hole was displaced with the cement formulation to be tested using a freshly prepared core for each test. The cement formulation thereby filled the muddled hole in the core. The cement formulation was

Table VIII

| Mix No.         | Composition of Mixtures |           |                                         |                  |      |                                                 |      |                                     |                              |            |            |        | Bonding Strength         |       |      |      |                  |
|-----------------|-------------------------|-----------|-----------------------------------------|------------------|------|-------------------------------------------------|------|-------------------------------------|------------------------------|------------|------------|--------|--------------------------|-------|------|------|------------------|
|                 | Aluminous Material      |           | Lbs. 85% H <sub>3</sub> PO <sub>4</sub> | Fluoride         |      | Sulfate                                         |      | Lbs. As <sub>2</sub> O <sub>3</sub> | Lbs. Dispersant <sup>1</sup> | Water      |            | Ratios |                          |       |      |      |                  |
|                 | No. in Table I          | Lbs. Used |                                         | Kind             | Lbs. | Kind                                            | Lbs. |                                     |                              | Lbs. Added | Lbs. Total | Al/P   | Total H <sub>2</sub> O/P | F/P   | ° F. | Hrs. | P.s.i.           |
| 43              | 21                      | 2,400     | 1,671                                   |                  |      |                                                 |      | 12                                  | 45                           | 1,424      | 2,104      | 1.35   | 8.1                      |       | 175  | 72   | 15               |
| 44              | 21                      | 2,400     | 1,671                                   | CaF <sub>2</sub> | 750  |                                                 |      | 12                                  | 45                           | 1,424      | 2,104      | 1.36   | 8.1                      | 1.33  | 175  | 72   | 162              |
| 45              | 22                      | 2,400     | 1,671                                   | CaF <sub>2</sub> | 750  | K <sub>2</sub> SO <sub>4</sub>                  | 600  | 6                                   | 45                           | 1,424      | 1,984      | 1.2    | 7.6                      | 1.33  | 175  | 72   | 39               |
| 46              | 22                      | 2,400     | 1,671                                   |                  |      | K <sub>2</sub> SO <sub>4</sub>                  | 600  | 6                                   | 45                           | 1,424      | 1,984      | 1.2    | 7.6                      |       |      |      | ( <sup>2</sup> ) |
| 47              | 22                      | 2,400     | 1,671                                   | KHF <sub>2</sub> | 30   |                                                 |      | 6                                   | 45                           | 1,424      | 1,984      | 1.2    | 7.6                      | 0.053 | 175  | 72   | 110              |
| 48              | 22                      | 2,400     | 1,671                                   | KHF <sub>2</sub> | 300  |                                                 |      | 6                                   | 45                           | 1,424      | 1,984      | 1.2    | 7.6                      | 0.53  | 175  | 72   | 108              |
| 49              | 22                      | 2,400     | 1,671                                   | CaF <sub>2</sub> | 750  | H <sub>2</sub> SO <sub>4</sub>                  | 342  | 6                                   | 45                           | 1,424      | 1,984      | 1.2    | 7.6                      | 1.33  | 175  | 72   | 108              |
| 50              | 22                      | 1,995     | 751                                     | CaF <sub>2</sub> | 503  | K <sub>2</sub> SO <sub>4</sub>                  | 390  | 6                                   | 45                           | 1,186      | 1,464      | 2.2    | 12.5                     | 2.12  | 175  | 72   | >70              |
| 51              | 4                       | 1,995     | 751                                     | KHF <sub>2</sub> | 37   | K <sub>2</sub> SO <sub>4</sub>                  | 390  | 6                                   | 30                           | 1,186      | 1,998      | 3.9    | 17.0                     | 2.12  | 175  | 72   | 81               |
| 52 <sup>2</sup> | 22                      | 960       | 751                                     | CaF <sub>2</sub> | 300  | K <sub>2</sub> SO <sub>4</sub>                  | 156  | 6                                   | 18                           | 1,186      | 1,320      | 1.07   | 11.2                     | 1.3   | 175  | 72   | 168              |
|                 |                         |           |                                         | KHF <sub>2</sub> | 30   | (NH <sub>4</sub> ) <sub>2</sub> SO <sub>4</sub> | 60   |                                     |                              |            |            |        |                          |       |      |      |                  |

<sup>1</sup> Polymerized sodium salts of alkyl naphthalene sulfonic acid.

<sup>2</sup> Contains 1,200 lbs. of powdered bituminous coal as a filler.

<sup>3</sup> Greater than specimen which broke in test.

then pressed against the mudded wall of the hole by applying a pressure of 200 p. s. i. to the formulation in the core. During the application of this pressure, the core was maintained at 175° F. for 48 hours while the cement was thereby hardened in situ.

After the cement formulations had set, the cores so-prepared were cut into short lengths. This was accomplished by sawing each core in a plane perpendicular to the axis. The length of the sections so-obtained was from 1 to 4 inches. The sections so-obtained comprised an annular ring of core with a solid cylindrical plug of cement bonded to the inside through the mud cake. The bonding strength was measured by ascertaining the force required to break the bond between the cement and the inside of the core section on pushing out the solid plug of cement. The force in pounds thus measured divided by the area in square inches of the inside of the section of core is the figure recorded in Table VIII as the bonding strength in p. s. i.

Similar tests were made with Portland cement for comparison. In these tests the Portland cement solidified in the mudded hole of the core in each instance as a more or less cylindrical chunk separate from and unbonded to the wall of the hole. The chunk of Portland cement fell out of each core on being sectioned. There was no evidence of bonding.

Referring to Table VIII, showing bonding strength measurements, mix 43 is an example of a cement formulation using an aluminous material and phosphoric acid, without additaments other than a corrosion inhibitor ( $As_2O_3$ ) and a dispersant. The bonding strength is that obtained in the test above described after allowing the mix to set for 72 hours. The bonding strength of the formulation of the kind illustrated by mix number 43 is improved by the addition to the mix of  $CaF_2$  as exemplified by mix number 44 using the same aluminous material as mix number 43. Mix number 45 is illustrative of the bond strength of a similar mix to that of number 44 but using a different aluminous material and containing  $K_2SO_4$ . With this aluminous material (#22) potassium sulfate in the formulation is illustrated in mix number 46. A much smaller proportion of  $KHF_2$  in place of  $CaF_2$  or  $K_2SO_4$  improves the bond as exemplified by mix number 47. In mix 47 the ratio of F/P is 0.053; larger amounts of  $KHF_2$ , as in mix 48, in which the ratio F/P is 0.53, produce about the same strength of bond. The combined use of calcium fluoride and sulfuric acid as in mix number 49 produces substantially the bonding strength obtainable with  $KHF_2$  as the sole source of fluorine but with the advantage of lower cost. Mixes having a high bonding strength and other desirable characteristics may contain three additaments, exclusive of the corrosion inhibitor and the dispersant, e. g.  $CaF_2$ ,  $KHF_2$ , and  $K_2SO_4$ . Examples are mix numbers 50 and 51 using different aluminous materials. Improved bonding results on including in the mixes the combination of the sulfates of ammonium and potassium along with  $CaF_2$  and  $KHF_2$ . An example of such a mix is number 52. Either the corrosion inhibitor or the dispersant or both may be omitted without substantially affecting the bonding action.

The presence of potassium salts, such as potassium sulfate and potassium phosphate or ammonium salts, such as ammonium sulfate and ammonium hydrogen phosphate, for example, in concentrations of about 1 to 15 percent by weight, like soluble fluoride, enables the cement formulation of the aluminous material and phosphoric acid to resist heat softening up to a temperature of at least 500° F. Such cement formulations are especially advantageous in cementing casing in very deep wells the earth formation of which is excessively hot. The following four mixes, 53 to 56 inclusive, are examples of a cement of this kind. The mixes are made by mixing together the listed ingredients.

|   | Mix No. 53:                       | Pounds |
|---|-----------------------------------|--------|
| 5 | Aluminous material #10 of Table I | 120    |
|   | Phosphoric acid (85%)             | 66.9   |
|   | Water                             | 56.9   |
|   | Potassium sulfate                 | 24.0   |

At 130° F. the mixture sets in less than 10 hours. At 78° F. it sets in about 71 hours. On being aged at 130° F. 144 hours after setting, the aged mixture may be heated to 500° F. without softening.

|    | Mix No. 54:                      | Pounds |
|----|----------------------------------|--------|
| 15 | Aluminous material #4 of Table I | 45     |
|    | Phosphoric acid (85%)            | 45     |
|    | Ammonium hydrogen phosphate      | 10     |

On mixing the foregoing ingredients at 212° F. in the order listed, the mixture resists softening on heating to 500° F. after ageing for 72 hours at 78° F.

|    | Mix No. 55:                       | Pounds |
|----|-----------------------------------|--------|
| 25 | Aluminous material #4 of Table I  | 33     |
|    | Phosphoric acid (85%)             | 60     |
|    | Potassium phosphate ( $K_3PO_4$ ) | 7      |

On mixing the foregoing ingredients at 212° F. in the order listed, the mixture resists softening on heating to 500° F. after ageing for 72 hours at 78° F.

|    | Mix No. 56:                      | Pounds |
|----|----------------------------------|--------|
| 35 | Aluminous material #4 of Table I | 39     |
|    | Phosphoric acid (85%)            | 46     |
|    | Potassium bifluoride ( $KF.HF$ ) | 15     |

On mixing the foregoing ingredients at 78° F. in the order listed, the mixture resists softening on heating to 500° F. after ageing at 78° F. for 72 hours.

Although mix numbers 54 and 55 were prepared at 212° F. lower temperatures may be employed such as those ordinarily prevailing at the earth's surface.

In addition to the advantageous effects on preventing heat-softening already mentioned, the ions of K and  $NH_4$  in the cement formulations give rise to improved properties particularly as regards compressive strength and especially when used in formulations containing also a soluble fluoride. The amount of potassium or ammonium employed may produce a ratio of K or  $(NH_4)$  to P in the mixtures of up to 3. A generally useful range for the ratio is between 0.2 and 2.0.

As already indicated, certain additaments added to the cement formulation in particular combinations are especially advantageous. Among such combinations of additaments contemplated by the invention are potassium sulfate and potassium bifluoride; potassium sulfate and ammonium bifluoride; calcium fluoride and potassium sulfate; calcium fluoride, potassium sulfate and ammonium bifluoride; potassium bifluoride and potassium phosphate; potassium bifluoride and ammonium phosphate. Some examples of the combined use of such additaments appear in previous tables.

By using various amounts of potassium bifluoride in combination with potassium sulfate in cement formulations comprising the aluminous material, phosphoric acid, and calcium fluoride, with or without the inclusion of a filler, a wide range of setting times together with bonding to the earth and high strength may be had at the temperatures encountered in deep wells.

The slurries of the cements herein comprising a clay exhibit a gel strength of from about 200 to 600 grams measured in accordance with the standard procedure used

in testing drilling muds. As made, such slurries immediately gel more or less but upon agitation the gel strength decreases. It is desirable to include in such slurries, in order to reduce their gel strength, a water- and acid-soluble anionic dispersing agent, such as an alkyl aryl sulfonate or alkali metal salt thereof. Some of the formulations already exemplified contain a dispersant as indicated. The amount which may be added is not critical since the effect on the gel strength is more or less proportional to the amount used up to about 3 percent by weight of the slurry. Lesser amounts produce a lesser effect on gel strength reduction. For example, a slurry composed of 43.7 pounds of kaolinitic clay (No. 21 of Table I), 37.6 pounds of 85 percent phosphoric acid, 14.9 pounds of calcium fluoride, 11.2 pounds of  $K_2SO_4$ , 1.8 pounds of  $KHF_2$ , 53.6 pounds of water, and 59.7 pounds of pulverized bituminous coal, as a filler, has an initial gel strength of 275 grams; after 10 minutes of standing the gel strength increases to 300 grams. On adding to the slurry 0.4 percent of the sodium salt of naphthalene sulfonic acid condensed with formaldehyde (Tamol N), the initial gel strength is only 35 grams and on standing for 10 minutes the gel strength increases only to 50 grams. Other examples of suitable dispersing agents are the polymerized sodium salts of alkyl naphthalene sulfonic acid (Daxad 11); the sodium salt of polymerized alkyl aryl sulfonic acid condensed with formaldehyde (Darvan 1); the high molecular weight alkyl aryl sodium sulfonates (Naccotan A). The dispersing agents which are used to decrease the gel strength do not adversely affect the cementing action of the slurries.

In cementing wells using the more complex formulations, it is advantageous to mix together first the aluminous material, phosphoric acid (more or less diluted with water) and filler if used. If calcium fluoride is to be included in the formulation, it may be added along with the aluminous material. The mixture so-prepared sets more or less slowly largely depending upon the temperature and activity of the aluminous material which may be chosen for the formulation so that plenty of time is available in which to incorporate the other additaments. At about the time the well is to be cemented, the other additaments of the formulation may be added as desired and mixed in thoroughly. These other additaments may comprise soluble fluoride which speeds up the setting time and potassium sulfate which promotes greater strength. Ammonium sulfate may be added also if desired. At this stage, a dispersant may be added to the mixture so as to reduce the gel strength and thereby facilitate pumping. The mixture is then ready for injection into the well in the usual way to cement the casing.

The amount of filler the mixtures can tolerate varies over a wide range and depends to some extent upon the bulkiness of the aluminous material used and the degree of fluidity it is desired the mixtures should have. In general the amount of filler will not exceed about 200 percent of the weight of the aluminous material. For example a generally useful amount to use with a bauxite as the aluminous material is a weight of about 125% of that of the bauxite. With a kaolin as the aluminous material, the filler may amount to as much as 150 percent of the weight of the kaolin.

The following mixes of general utility and preferred composition are examples of cement formulations designed for use over three ranges of temperature most commonly encountered in the well. These mixes are most advantageously prepared by mixing together in powder form certain of the dry ingredients, viz. the aluminous material, filler, calcium fluoride, potassium sulfate, and dry powdered dispersant, if used, so as to form a dry mix. The dry mix may be put up in sacks or other convenient form of package suitable for storage or transportation. The dry mix may be transported to

the site of the cementing operation and there mixed with phosphoric acid and water to form a fluid self-hardening slurry. The addition of soluble fluoride (e. g.  $KHF_2$ ), which speeds up the setting rate, is incorporated in the mixture as desired following the addition of the phosphoric acid and water. The mixture so-prepared is then ready for use in the cementing operation and will set within a time predetermined by the kinds and proportions of the ingredients. At the temperature for which the mixture is designed, other things being equal, the lapse of time before setting occurs depends upon the amount of soluble fluoride added. Examples of three dry formulations, mix A, B, and C, are set forth in the following Table IX.

Table IX

|    | Designation                           | Dry Mix A    | Dry Mix B                        | Dry Mix C    |
|----|---------------------------------------|--------------|----------------------------------|--------------|
|    | Temp. Range... ° F...                 | 60 to 130    | 100 to 140                       | 130 to 200   |
| 25 | Materials, Lbs.:                      |              |                                  |              |
|    | Aluminous Material <sup>1</sup> ..... | No. 10, 41.0 | { No. 10, 12.8<br>No. 22, 25.6 } | No. 22, 35.6 |
|    | Filler, coal.....                     | 41.0         | 42.8                             | 44.8         |
|    | Fluorospar, $CaF_2$ .....             | 10.2         | 10.7                             | 11.2         |
|    | $K_2SO_4$ .....                       | 7.2          | 7.5                              | 7.8          |
|    | Dispersant <sup>2</sup> .....         | 0.6          | 0.6                              | 0.6          |
| 30 | Total weight...                       | 100.0        | 100.0                            | 100.0        |

<sup>1</sup> No. in Table I.

<sup>2</sup> Polymerized sodium salts of alkyl naphthalene sulfonic acid.

Referring to Table IX, it will be observed that each dry mixture is compounded of a different aluminous material. Mixes A and C employ aluminous materials 10 and 22, respectively, and mix B employs a mixture of 10 and 22. Each dry mix is designed to provide a cement for use over a different range of temperature. The ranges overlap somewhat and cover most of the temperatures encountered in well cementing operations. Such dry formulations, and in particular those of Table IX, may be mixed with diluted phosphoric acid (phosphoric acid and water) using an appropriate amount thereof to form a cementing slurry as shown in Table X.

Table X

|    | Lbs. of Water and 85% $H_3PO_4$ to Add Per 100 Lbs. of Dry Mix |              |              |              |
|----|----------------------------------------------------------------|--------------|--------------|--------------|
|    | Dry Mix A                                                      | Dry Mix B    | Dry Mix C    |              |
| 60 | $H_2O$ .....<br>85% $H_3PO_4$ .....                            | 27.6<br>23.1 | 25.6<br>27.7 | 26.2<br>28.1 |

The rate of setting of the slurries at a given temperature is accelerated as aforesaid by the addition of soluble fluoride. The amount used is selected according to the setting time desired at the temperature at which cementing is to be performed. As illustrative of this, data are set forth in Table XI showing the amount of  $KHF_2$  to incorporate in the slurries based upon the weight of dry mixtures to provide a wide range of predetermined slurry setting times at the temperatures indicated.

Table XI

| KHF <sub>2</sub> , Lbs. Per 100<br>Lbs. of Dry Mix | Mix A                       |     | Mix B |       | Mix C |     |       |     |     |       |
|----------------------------------------------------|-----------------------------|-----|-------|-------|-------|-----|-------|-----|-----|-------|
|                                                    | Temperature of Setting, °F. |     |       |       |       |     |       |     |     |       |
|                                                    | 78                          | 90  | 110   | 130   | 110   | 130 | 150   | 150 | 180 | 194   |
| Hours of Setting Time                              |                             |     |       |       |       |     |       |     |     |       |
| 0.31                                               | 35                          | 15  | 5.5   | 2.4   | 9     | 4.4 | 2.2   | 15  | 3.8 | 2.6   |
| 0.62                                               | 24                          | 11  | 4.0   | 1.7   | 7     | 3.2 | 1.7   | 11  | 3.0 | 2.0   |
| 1.25                                               | 14                          | 7   | 2.5   | 1.0   | 4.4   | 2.0 | 1.1   | 5.5 | 1.7 | 1.1   |
| 1.87                                               | 9.5                         | 5   | 1.7   | 0.6   | 3.0   | 1.4 | 0.7   | 2.8 | 0.9 | 0.6   |
| 2.5                                                | 7                           | 3.7 | 1.2   | ----- | 2.2   | 1.0 | ----- | 1.6 | 0.6 | ----- |

Although the invention has been described more particularly with reference to forming a monolithic body as a seal between the wall of a well hole in the earth and a well casing therein, it will be apparent that sealing deposits can also be formed in an uncased portion of a well hole as for example in the hole below a casing, or other hole in the earth, where the cement formulation may be brought into contact with and set against an earth surface.

Among the advantages of the invention are that the rate at which sealing or setting of the cement *in situ* may be brought about is subject to a wide range of control; the method is usable over the wide range of temperatures encountered in the earth formations penetrated by wells to be cemented; the cement formulation on being deposited in a well hole resist loss, by filtration, of its liquid portion and thus remains pumpable under adverse well conditions in which other cements suffer a damaging liquid loss; drilling mud and drilling mud additaments are tolerated by the cement formulations to an extent which does not prevent obtaining a proper seal between the well hole and the well casing therein; the cementing method produces a true bond with the mudded wall of the well hole in an earth formation; fillers may be included in the formulations for lowering the cost, and for reducing or increasing the density as desired; the cement formulations are easily and rapidly prepared and injected without difficulty by pumping into the well.

We claim:

1. The method of cementing a well formed in the earth which comprises depositing therein into contact with the earth formation a flowable self-hardening mixture consisting of an aluminous material in particulate form selected from the group consisting of the oxides, hydroxides, and silicates of aluminum, phosphoric acid, and water, the ratio of the number of moles of aluminum (Al) to the number of moles of phosphorus (P) in the mixture being between 0.5 and 20, and the ratio of the number of moles of water (H<sub>2</sub>O) to the number of moles of phosphorus (P) in the mixture being between 1.8 and 64.

2. The method according to claim 1 in which there is incorporated in the mixture a filler of a particulated solid unreactive with the phosphoric acid and the aluminous material.

3. The method according to claim 1 in which the mixture includes an inorganic fluorine compound.

4. The method according to claim 1 in which the mixture includes a water-soluble inorganic fluoride selected from the group consisting of ammonium fluoride, ammonium bifluoride, potassium fluoride, potassium bifluoride, and hydrogen fluoride.

5. The method according to claim 1 in which the mixture includes a water-soluble inorganic sulfate and calcium fluoride.

6. The method according to claim 1 in which the mixture includes calcium fluoride and a water-soluble sulfate selected from the group consisting of K<sub>2</sub>SO<sub>4</sub>, H<sub>2</sub>SO<sub>4</sub>, and (NH<sub>4</sub>)<sub>2</sub>SO<sub>4</sub>, and a water-soluble fluoride selected from the group consisting of ammonium fluoride, ammonium bifluoride, potassium fluoride, potassium bifluoride, and hydrogen fluoride.

from the group consisting of ammonium fluoride, ammonium bifluoride, potassium fluoride, potassium bifluoride, and hydrogen fluoride.

7. The method according to claim 1 in which the mixture includes calcium fluoride, potassium sulfate, and potassium fluoride, and the ratio of F/P is between 0.02 and 10.

8. The method according to claim 3 in which the ratio of the number of moles of fluorine (F) derived from the fluorine compound to the number of moles of phosphorus (P) derived from the phosphoric acid is between 0.02 and 10.

9. The method according to claim 3 in which the fluorine compound is selected from the group consisting of the fluophosphoric acids, potassium fluotitanate, ammonium fluotitanate, ammonium fluosilicate, potassium fluosilicate, potassium borofluoride, potassium fluorochromite.

10. The method according to claim 7 in which the ratio of K/P is between 0.2 and 3 and the mixture includes ammonium sulfate.

11. The method according to claim 1 in which the mixture includes aluminum fluoride, and a water-soluble sulfate selected from the group consisting of K<sub>2</sub>SO<sub>4</sub>, H<sub>2</sub>SO<sub>4</sub>, and (NH<sub>4</sub>)<sub>2</sub>SO<sub>4</sub>, and a water-soluble fluoride selected from the group consisting of ammonium fluoride, ammonium bifluoride, potassium fluoride, potassium bifluoride, and hydrogen fluoride.

12. The method according to claim 1 in which the mixture includes calcium fluoride, potassium sulfate, and potassium bifluoride, and the ratio of F/P is between 0.02 and 10.

13. The method of forming a fluid mixture capable of hardening into a monolithic body which consists in mixing together an aluminous material in particulate form selected from the group consisting of the oxides, hydroxide and silicates of aluminum, phosphoric acid, and water so as to produce a fluid slurry in which the ratio of Al to P is between 0.5 and 20 and the ratio of H<sub>2</sub>O to P is between 1.8 and 64, and incorporating in the slurry an inorganic fluorine compound selected from the group consisting of ammonium fluoride, ammonium bifluoride, potassium fluoride, potassium bifluoride, and hydrogen fluoride in amount sufficient to provide therein a ratio of F to P of from 0.02 to 10.

14. The method according to claim 13 in which there is included in the slurry a water-soluble inorganic sulfate and calcium fluoride.

15. The method according to claim 14 in which the water-soluble inorganic sulfate is potassium sulfate in amount sufficient to produce therein a ratio of K/P of up to 4.

16. The method according to claim 14 in which the water-soluble inorganic sulfate is ammonium sulfate and is present in amount sufficient to produce therein a ratio of NH<sub>4</sub>/P of up to 4.

17. The method according to claim 13 in which the fluorine compound is selected from the group consisting of the fluophosphoric acids, potassium fluotitanate, ammonium fluotitanate, ammonium fluosilicate, potassium

fluosilicate, potassium borofluoride, potassium fluochromite.

18. A self-hardening mixture consisting of a water-insoluble naturally occurring aluminous material in particulate form containing at least 7 percent of  $\text{Al}_2\text{O}_3$  by weight, phosphoric acid in amount sufficient to provide in the mixture a ratio of Al/P of between 0.5 and 20, a fluorine compound selected from the group consisting of potassium fluoride, potassium bifluoride, the fluophosphoric acids, ammonium fluoride, ammonium bifluoride, hydrogen fluoride, potassium fluotitanate, ammonium fluotitanate, ammonium fluosilicate, potassium fluosilicate, potassium borofluoride, potassium fluochromite in amount sufficient to provide a ratio of F/P of between 0.02 and 10, and water including that, if any, occurring with the aluminous material, phosphoric acid and the fluoride, in amount sufficient to provide a ratio of  $\text{H}_2\text{O}/\text{P}$  of between 1.8 and 64.

19. A self-hardening mixture according to claim 18 including a water-soluble inorganic sulfate in amount between 1 and 15 percent by weight, and calcium fluoride in amount between 2 and 20 percent by weight of mixture.

20. A self-hardening mixture according to claim 18 including a soluble sulfate selected from the group consisting of ammonium sulfate and potassium sulfate in amount between 1 and 15 percent by weight, and calcium fluoride in amount between 2 and 20 percent by weight of the mixture.

21. The method according to claim 13 in which there is included in the slurry a water-soluble inorganic sulfate selected from the group consisting of  $\text{K}_2\text{SO}_4$ ,  $\text{H}_2\text{SO}_4$ , and  $(\text{NH}_4)_2\text{SO}_4$  and aluminum fluoride.

22. A self-hardening mixture according to claim 18 including a water-soluble inorganic sulfate in amount between 1 and 15 percent by weight, and aluminum fluoride in amount between 2 and 20 percent by weight of the mixture.

23. A self-hardening mixture according to claim 18 including a soluble sulfate selected from the group consisting of ammonium sulfate and potassium sulfate in amount between 1 and 15 percent by weight, and alu-

minum fluoride in amount between 2 and 20 percent by weight of the mixture.

24. The method according to claim 1 in which the aluminous material is clay.

25. A dry formulation capable of forming a self-hardening mixture on being mixed with phosphoric acid and water to form a flowable slurry consisting of a mixture of 10.2 to 11.2 parts by weight of calcium fluoride; from 35.6 to 41 parts of bauxite; and from 7.2 to 7.8 parts of potassium sulfate.

26. A dry formulation capable of forming a self-hardening mixture on being mixed with phosphoric acid and water to form a flowable slurry consisting of a mixture of 10.2 to 11.2 parts by weight of calcium fluoride; from 35.6 to 41 parts of kaolinitic clay; and from 7.2 to 7.8 parts of potassium sulfate.

27. A dry formulation capable of forming a self-hardening mixture on being mixed with phosphoric acid and water to form a flowable slurry consisting of a mixture of 10.2 to 11.2 parts by weight of calcium fluoride; from 35.6 to 41 parts of vermiculite; and from 7.2 to 7.8 parts of potassium sulfate.

#### References Cited in the file of this patent

##### UNITED STATES PATENTS

|           |                   |       |               |
|-----------|-------------------|-------|---------------|
| 225,817   | Fletcher          | ----- | Mar. 23, 1880 |
| 1,507,379 | Hoskins           | ----- | Sept. 2, 1924 |
| 1,556,115 | Hoskins           | ----- | Oct. 6, 1925  |
| 1,908,636 | Langenberg et al. | ----- | May 9, 1933   |
| 2,146,480 | Kennedy           | ----- | Feb. 7, 1939  |
| 2,188,767 | Cannon            | ----- | Jan. 30, 1940 |
| 2,218,058 | Stalhane          | ----- | Oct. 15, 1940 |
| 2,285,302 | Patterson         | ----- | June 2, 1942  |
| 2,391,493 | Wainer            | ----- | Dec. 25, 1945 |
| 2,450,952 | Greger            | ----- | Oct. 12, 1948 |
| 2,562,148 | Lea               | ----- | July 24, 1951 |

##### FOREIGN PATENTS

|               |       |               |
|---------------|-------|---------------|
| Great Britain | ----- | of 1907       |
| Great Britain | ----- | Dec. 24, 1935 |